

## UNITED STATES PATENT OFFICE.

CAMILLE DREYFUS, OF BASEL, SWITZERLAND, ASSIGNOR TO CELANESE CORPORATION OF AMERICA, A CORPORATION OF DELAWARE.

## MANUFACTURE OF KNITTED FABRICS AND ARTICLES.

No Drawing.

Application filed February 23, 1924. Serial No. 694,810.

Fabrics and articles when made, for instance, on a circular knitting machine or on a knitting machine of circular knitting type or other knitting machine, are more or less 5 subject to laddering, which is a very big draw-back.

It has now been found that this laddering feature in fabrics and articles can be completely or partly eliminated or substantially 10 reduced by impregnating or treating the fabric or article which ladders with a material (which material can be a gas or a solvent or a liquid or a solution of a solid in a liquid, etc.) having the effect of binding 15 more or less threads or filaments of threads together in the fabric or article or melting more or less threads or filaments together of the fabric or article, thus creating a resistance to laddering. These substances are 20 preferably chosen in such a composition or solution, etc., or are applied in such a way as not to interfere substantially with the texture or with the nature or appearance of the fabrics or articles so produced.

25 The invention can be carried out with fabrics or articles made of fibres or mixtures of fibres, such as cotton, wool, silk, artificial silks, yarns, artificial silks made from organic or inorganic derivatives of cellulose, 30 such as cellulose acetate or ethers or esters of cellulose or nitro cellulose and others or from mixtures of different fibres.

35 *Example #1.*—Knitted silk fabrics or articles of silk subject to laddering are treated with alkali or acetic acid in such a strength as to just attack the fibres slightly and melt or stick them slightly and superficially together.

40 *Example #2.*—Knitted fabrics or articles made from cellulose acetate artificial silk, or from cellulose ether silk, or from other organic or inorganic derivatives of cellulose, subject to laddering, are treated with acetone (in gas form or as a liquid or with 45 other solvents in such a diluted composition with air or with water or other diluents so as not to interfere substantially with the texture or appearance or nature of the fabric or

article, in an analogous way and with a similar result as under Example 1. 50

The above examples are only some representative examples to show the way this invention can be carried out, but this invention is not limited to the above examples and any suitable material, substance, solution, gas, 55 air, diluents, with or without the use of any suitable mechanical device, can be used for the execution of this invention.

What I claim is:

1. Process for the treatment of knitted fabrics and articles containing fibres of organic derivatives of cellulose for the purpose of reducing tendency to laddering, said process comprising treating the fabric or article with an agent having a slight solvent 60 action on the organic derivative of cellulose fibres composing the threads, whereby the fibres and threads are caused to adhere slightly together in the knit web without substantially affecting the texture and appearance of the web. 65

2. Process for the treatment of knitted fabrics and articles composed of threads of cellulose acetate artificial silk, for the purpose of reducing tendency to laddering, said 70 process comprising treating the fabric or article with a solvent of cellulose acetate in a dilution capable of exerting only a slight solvent action on the cellulose acetate fibres whereby the fibres and threads are caused to 75 adhere slightly together in the knit web without substantially affecting the texture and appearance of the web.

3. Process for the treatment of knitted fabrics and articles composed of threads of an organic derivative of cellulose, for the purpose of reducing tendency to laddering, said process comprising treating fabric or articles with a solvent of said cellulose derivative in a dilution capable of exerting 80 only a slight solvent action on the fibres of said cellulose derivative whereby the fibres and threads are caused to adhere slightly together in the knit web without substantially 85 affecting the texture and appearance of the web. 90

95

4. Knitted fabrics and articles of cellulose acetate whose contiguous fibres adhere slightly to each other throughout the web and in which the web substantially retains its original texture and appearance.

5. Knitted fabrics and articles of an organic cellulose derivative whose contiguous fibres adhere slightly to each other through-

out the web and in which the web substantially retains its original texture and appearance. 10

In testimony whereof, I have hereunto subscribed my name this 21st day of February, 1924.

**CAMILLE DREYFUS.**